

Jan. 10, 1950

J. H. BUCKNAM ET AL  
PROCESS OF THERMOCHEMICALLY  
CONDITIONING METAL BODIES  
Filed May 10, 1949

2,493,802



Fig. 1.



<sup>5</sup> Fig. 2.



1

INVENTORS  
JAMES H. BUCKNAM  
IVAN P. THOMPSON  
*El Greenerwald*  
ATTORNEY

## UNITED STATES PATENT OFFICE

2,493,802

## PROCESS OF THERMOCHEMICALLY CONDITIONING METAL BODIES

James H. Bucknam, Cranford, and Ivan P. Thompson, Elizabeth, N. J., assignors to The Linde Air Products Company, a corporation of Ohio

Application May 10, 1949, Serial No. 92,274

3 Claims. (Cl. 148—9.5)

1

This application is a continuation-in-part of application Serial No. 478,202, filed March 6, 1943 for Blowpipe nozzle, which was patented on August 19, 1947, No. 2,425,709; and of abandoned application Serial No. 517,472, filed January 7, 1944 for Process of thermochemically conditioning metal bodies.

The invention relates to the art of thermochemically conditioning metal bodies and, more particularly, to the removal of surface defects in ferrous metal bodies with an oxidizing stream and in conjunction with externally mixed excess-oxygen oxy-acetylene preheating flames.

Above a red heat, iron combines with pure oxygen so rapidly that it actually burns. Thus, if a spot on a piece of iron or steel is heated to the kindling temperature, and a jet of oxygen is directed against such heated spot, the iron will begin to burn vigorously with the generation of heat. Although the result of this combination of iron and oxygen is the formation of iron oxide, a product that is solid at ordinary temperatures, the iron oxide melts at a temperature somewhat below the melting point of iron or steel. During oxy-acetylene cutting, the heat generated by the burning iron is sufficient to melt the iron oxide so that it runs off as a molten slag, not only exposing more iron to the action of the oxygen jet but also carrying away with it some iron that has become molten at the temperature of the operation, but which has not actually become oxidized.

Radiation at the surface, pieces of dirt or scale on the metal, and the fact that heat is conducted into the metal body when cold, make it necessary for additional heat to be supplied or the cut will stop or be lost. It is customary, therefore, to provide a blowpipe nozzle having small orifices for oxy-acetylene heating flames surrounding an opening that supplies the cutting oxygen jet or stream. In making a cut, such preheat flames are used to heat a spot to a red heat, and the cut is started by opening a valve controlling the oxygen jet and directing the stream of oxygen at the heated spot. The preheating flames remain burning while cutting is in progress to make up for the heat that is lost during the operation. It is thus seen that the thermochemical cutting of ferrous metal is a thermochemical reaction.

The thermochemical removal of surface defects in steel bodies during manufacture is accomplished by a process variously known as deseaming, scarfing, or conditioning. Generally, however, the term "deseaming," that is, the removal of surface seams or cracks, is used when the operation is performed with a hand blowpipe, only those defects being removed that are apparent on the surface of the metal body.

5

10

15

20

25

30

35

40

45

2

In mechanized steel conditioning, a shallow layer of the entire surface of the billet, bloom, or slab, is removed by a conditioning machine located in the rolling mill line. Such machine removes a thin layer containing surface defects from one, two, or four sides of the body simultaneously and the operation is performed while the metal is still hot and without interrupting the rolling operation. Secondary conditioning involving the removal of deeper defects generally is performed by hand deseaming after the steel has cooled down.

Prior to the present invention, oxy-acetylene scarfing machines for removing surface defects from semi-finished steel bodies consisted of mechanized batteries of oxy-acetylene blowpipes comprising mixers for premixing oxygen and acetylene for producing the preheating flames. Such mixers are not only expensive to manufacture and maintain, but they produce an oxy-acetylene gas mixture that is highly combustible, rendering the machines subject to backfire. A backfire is an explosion of the gases within the apparatus which may be caused by overheating of the apparatus, improper gas pressure, loose connections or unclean internal surfaces. In the event of a backfire, the affected machine parts must be taken apart for thorough cleaning, since a backfire fouls the interior of many of the parts with carbon. As a result, the gas hoses, valves, mixers, nozzles and other parts must be disassembled, repaired or replaced in case of damage, cleaned, reassembled and adjusted.

In order to avoid a backfire in desurfacing machines of the premixed oxy-acetylene preheating flame type, it is necessary to maintain all of the parts absolutely clean, tight and in proper adjustment. Even so, flashbacks occur, and each flashback requires replacement of the mixer, if burned out, as well as cleaning of the parts, so that the machine must be temporarily taken out of operation. In any case, the tendency of premixed oxy-acetylene desurfacing equipment to backfire presents a serious maintenance problem especially in the scarfing of hot steel. The principal object of this invention, therefore, is to solve such problem.

Desurfacing machines of the premixed oxy-acetylene preheating flame type are also subject to the objection that the inner cones of the premixed oxy-acetylene preheating flames are relatively short, being of the order of  $\frac{3}{8}$  to  $\frac{1}{2}$  inch long, and since the face of each nozzle is about  $\frac{1}{16}$  inch at its center from the surface undergoing conditioning, such face being at an angle with such surface, the ends of such inner cones do not impinge against such surface but are always

spaced a substantial distance, that is to say, at least  $\frac{1}{2}$  inch, away from such surface. Since the hottest part of a premixed oxy-acetylene flame is at the surface of the inner cone, it follows that the most efficient heating result cannot be obtained with such flames for desurfacing. Another object of the invention, therefore, is to provide an oxy-acetylene preheating flame that is more efficient and effective for starting and carrying on a thermochemical metal removal operation.

Prior desurfacing machines of the premixed oxy-acetylene preheating flame type employing a series of nozzles produce a conditioned surface that generally has low parallel ridges between the cuts. It is desirable to have such ridges as low or flat as possible, the ideal conditioned surface being one that is flat or entirely ridge-free. Therefore, another object of the invention is to provide a novel desurfacing process which produces a conditioned surface which is flatter and of better quality than those produced by prior processes.

Desurfacing equipment in the past has also been very expensive to manufacture and maintain, owing to the large number of complicated parts, including mixers and valves, that are involved. A further object of this invention is to provide an improved process to simplify the required equipment for desurfacing, entirely eliminating the mixers and as many control valves and other parts as possible.

Other important objects of the invention are to increase the metal removal efficiency of the oxygen, to reduce the preheating period for initial starting, to obtain faster cuts especially with cold steel, and to improve the stability of the operation.

According to the present invention, an entirely novel post-mixed excess-oxygen oxy-acetylene flame comprising a stream of oxygen is first applied against a preselected spot on the surface of the metal body. The excess oxygen in such flame causes the metal in the spot to become luminous at the very instant the temperature of such metal is raised to the ignition point. The body is then moved with respect to the flame (or the flame is moved with respect to the body), and the velocity of the oxygen stream is increased to a desurfacing value at the approximate instant the movement of the body is started, in order to prevent any nicking or gouging of the work by such oxygen stream at the starting spot. The amount of acetylene supplied to the oxygen stream is not changed. As a result, the post-mixed preheating flame assists the oxygen stream in progressively removing or skinning metal from the surface of the body, molten slag containing oxides being caused to flow ahead of the zone of thermochemical reaction between the oxygen and the heated metal.

The post-mixed oxy-acetylene preheating flame for starting and carrying on the operation according to the invention is quite hard and intensely hot, the temperature even approaching that of a premixed flame, the inner cones of the post-mixed flame, however, being extended and applied directly against the surface of the body which is being conditioned. For preheating the work to start the operation, the post-mixed flames of the present invention have inner cones or primary combustion zones which extend about  $1\frac{1}{4}$  inch from the face of the nozzle, a decided improvement over the premixed type of preheating.

flames in which, at best, the inner cones are only about  $\frac{1}{2}$  inch long.

In desurfacing a hot steel body, the body is moved into position under the head or heads so that the edge of the body is in spaced relation to the line of contact of the flames with the body. In desurfacing a cold steel body, however, the body is backed into position so that the flames are applied directly against the edge or edges of the body. In either case, since the post-mixed flames contain an excess of oxygen, the temperature of ignition becomes visible much more quickly than in the case of premixed flames, and not only enables the operator to start the desurfacing movement of the body at the proper time, but also reduces the starting time compared with that of the premixed flames.

Referring to the drawings:

Fig. 1 is a fragmentary perspective view of a steel body in starting position under a battery of post-mixed nozzles in a head which is supplied with oxygen and acetylene according to the invention;

Fig. 2 is a similar view showing the body undergoing the thermochemical desurfacing operation;

Fig. 3 is an enlarged fragmentary cross-sectional view of the head and a post-mixed nozzle carrying out the present invention; and

Fig. 4 is a view in front end elevation of the nozzle shown in Fig. 3.

In the illustrated example, a desurfacing head H is provided with a plurality of blowpipe nozzles N. Each nozzle N comprises a tubular body member 11 having a central cutting oxygen passage 12 extending longitudinally therethrough. Such passage 12 includes a cylindrical inlet portion of constant diameter, a flared frusto-conical portion, a short cylindrical portion of constant diameter, and an outlet portion which gradually changes from circular to flat cross section, the discharge end of the passage being oblong as shown at 13, with its longer axis disposed parallel to the work surface. The passage 12 thus is adapted to discharge a characteristic desurfacing oxidizing gas stream 14 which is flat. The tubular body member 11 is also provided with a plurality of acetylene passages 15 arranged in spaced parallel relation to the longitudinal axis of the oxygen passage 12, the passages 15 terminating above and below the oxygen orifice 13 in inclined plane surfaces 16, 16 at the end of the member 11. The oxygen orifice 13 lies in a plane disposed at right angles to the longitudinal axis of the member 11, and at the bottom of a peripheral recess 17.

The gas inlet end of the tubular body member 11 also is provided with a pair of radially and longitudinally spaced frusto-conical annular seats 18 and 19, which are adapted to mate with corresponding seats 20 and 21 in the head H. The member 11 is also provided with an annular flange 23 which is engaged by a hollow screw 24 threaded in a socket 25 in a body 26 of the head H, for locating the nozzle N in proper position in the head. The nozzle is coupled to the body 26 so that the acetylene is delivered to the acetylene passages 15 and oxygen is delivered to the central oxygen passage 12 through an oxygen channel 27 and an acetylene channel 28 in such body.

The outer end of the body member 11 is provided with the bevelled surfaces 16 which cooperate with inner walls of an end cap 29 to provide upper and lower transverse acetylene distributing passages 30, 30 having slot-like outlets

31, 31 above and below the oblong oxygen orifice 13. The cap 29 comprises a cylindrical skirt 32 which fits the end portion 33 of the nozzle body 11, the edge of the skirt being bronze-welded or silver-soldered at 34 to the body to secure such parts together. The cap includes a bottom panel 35 which is relatively thick to inhibit deformation or damage in use. The bottom panel of the cap has a slot 36 corresponding in position to the oxygen orifice 13, the upper and lower walls of the slot being parallel to and outwardly offset with respect to the top and bottom edges of the peripheral recess or groove 17. The groove 17 causes eddy currents and thus provides a fringe of low velocity oxygen around the otherwise solid oxygen stream, for admixture with the acetylene discharged by the slots 31, to form a post-mixed oxy-acetylene preheating flame F, when the oxygen stream 14 is discharged at a desurfacing velocity; and prevents such flame from being blown out. With this arrangement, acetylene discharged by the acetylene slots 31 is directed inwardly from above and below against the single flat stream of oxygen 14 discharged by the central passage 12 as the latter leaves the discharge end of the nozzle.

While nozzles N of the type shown in the drawings and described above, are preferred, similar nozzles of the type disclosed and claimed in our Patents 2,425,709 and 2,425,710 may also be employed.

The body 26 of the head is provided with a row of the sockets 25 into each one of which a nozzle N is secured by the hollow screw 24. The head H is also provided with a removable shoe 37 having a row of openings 38, there being an opening through which each nozzle N projects. Each nozzle is provided with a packing ring 39 which is held in place against the inner wall of the shoe by a coiled compression spring 40 disposed around the nozzle and between the hollow screw 24 and an annular bearing member 41 that engages the packing ring 39. Thus, when a chamber 42 is filled with cooling water, leakage between the nozzles N and the openings 38 is prevented. The shoe 37 is also provided with an outer layer of heat and wear resistant metal such as "Stellite" alloy, having spaced runners 43 adapted to ride on the surface S of the work W.

The body 26 of the head H is supplied with oxygen through pipes 44, and with acetylene through pipes 45, having gas distributing headers 46 and 47, respectively. The acetylene header 47 is connected to a suitable acetylene supply source A by means including a conduit 48 containing a pressure regulator 49 and a normally closed valve 50. The oxygen header 46 is connected to suitable sources of oxygen OP and OD by means including a conduit 51 having two inlet pipes 52 and 53. The inlet pipe 52 contains a pressure regulator 54 and a normally closed valve 55. The inlet pipe 53 contains a pressure regulator 56, a normally closed valve 57, and a reverse flow check valve 58. The valves 50, 57 and 55 are each adapted to be opened by an armature 60 when a coil 61 is energized by an electric current. The regulators 49 and 56 are set to maintain the pressure of the acetylene and oxygen passing therethrough at a predetermined low value, between 3 and 4 pounds per square inch for example, so that when the valves 50 and 57 are open all of the nozzles N are supplied with oxygen and acetylene in sufficient quantity to form post-mixed oxy-acetylene flames. The regulator 54 is set to maintain the pressure of the oxygen passing there-

through at a predetermined high value, between 30 and 75 pounds per square inch for example, so that when the valve 55 is open all of the nozzles N are supplied with oxygen in sufficient quantity to discharge desurfacing oxygen streams.

The control circuit including the coils 61 is such that the preheating acetylene and oxygen valves 50 and 57 are opened at the same time. At the end of the starting preheating period the desurfacing oxygen valve 55 is opened. All of the valves are kept open until the desurfacing operation is completed, whereupon all of the valves are closed. The movement of the work W is automatically started at the approximate instant the desurfacing oxygen valve 55 is opened.

A ferrous metal body W is thermochemically conditioned according to the present process as follows: the body, supported by a roll R, is moved into a starting position with respect to the desurfacing head H and preheating oxygen and acetylene are supplied to all of the nozzles N. These gases mix externally to produce a post-mixed flame which is applied against a local surface portion of the body. Since the flame contains an excess amount of oxygen for complete combustion, the portion of the surface being preheated becomes visible at the instant it reaches the kindling temperature because of the reaction of such excess oxygen with the heated metal. This enables the operator to start movement of the body W exactly at the proper time, reducing the starting time and making the operation more uniform when applied to successive bodies. Shortly after movement of the body W is started, the velocity of the oxygen stream is increased to a desurfacing value for thermochemical reaction with the heated metal without changing the quantity of acetylene discharge from the nozzles. By maintaining the quantity of acetylene supplied to the nozzles unchanged, much control equipment is eliminated.

Acetylene is supplied to the nozzles at the rate of about 100 cubic feet per hour. During the starting preheat period oxygen is supplied to the nozzles at a slightly higher rate, resulting in a fairly efficient post-mixed oxy-acetylene flame, which contains an excess amount of oxygen for complete combustion of the acetylene. During the desurfacing operation oxygen is supplied to each of the nozzles at the rate of between 1700 and 4000 cubic feet per hour, the exact rate depending upon the composition of the metal and the depth of the conditioning desired. After the body has moved sufficiently to be desurfaced throughout its entire length the oxygen and acetylene are shut off.

#### Calculated acetylene flows

| Acetylene Pressure at Nozzle Seat, p. s. i. | Total Acetylene Flow Through Nozzle in c. f. h. | Velocity through each Rectangular Passage, f. p. s. | Velocity through each Drilling, f. p. s. |
|---------------------------------------------|-------------------------------------------------|-----------------------------------------------------|------------------------------------------|
| .49                                         | 52.4                                            | 139                                                 | 110                                      |
| .71                                         | 65.2                                            | 173                                                 | 137                                      |
| .85                                         | 75.0                                            | 199                                                 | 157                                      |
| 1.1                                         | 85.5                                            | 227                                                 | 180                                      |
| 1.7                                         | 108.0                                           | 287                                                 | 227                                      |
| 2.1                                         | 128.5                                           | 342                                                 | 271                                      |
| 2.6                                         | 138.2                                           | 368                                                 | 291                                      |
| 2.9                                         | 151.2                                           | 403                                                 | 318                                      |
| 3.4                                         | 165.9                                           | 441                                                 | 349                                      |

NOTE.—The above velocities are calculated from the formula

$$V = \frac{Q}{A}$$

Each of the six acetylene drillings 15 is 0.0635 inch in diameter and has an area of 0.003167 square inch.

Each of the two rectangular acetylene passages 31 at the end of the nozzles has a nominal area of 0.0075 square inch.

Normal operating range is from 90 to 100 cubic feet/hour (about 240-267 feet/second through passage 31).

#### Calculated oxygen flows

| Pressure<br>At Seat,<br>p. s. i. | Oxygen Flow,<br>c. f. h. | Vacuum on<br>Acetylene<br>Passage<br>In. Water | Velocity at<br>End of Nozzle<br>f. p. s. |
|----------------------------------|--------------------------|------------------------------------------------|------------------------------------------|
| 1.34                             | 206                      | 0                                              | 111                                      |
| 1.34                             | 302                      | 0.3                                            | 162                                      |
| 1.49                             | 336                      | 0.9                                            | 208                                      |
| 1.03                             | 513                      | 1.3                                            | 276                                      |
| 1.6                              | 636                      | 1.7                                            | 342                                      |
| 2.46                             | 790                      | 2.1                                            | 424                                      |
| 4.01                             | 992                      | 2.8                                            | 533                                      |
| 9.6                              | 1,315                    | 3.7                                            | 707                                      |
| 12.9                             | 1,490                    | 5.1                                            | 802                                      |
| 17.8                             | 1,756                    | 5.8                                            | 944                                      |
| 25.8                             | 2,200                    | 4.8                                            | 1,180                                    |
| 31.5                             | 2,505                    | 5.2                                            | 1,340                                    |
| 37                               | 2,802                    | 5.3                                            | 1,510                                    |
| 39.9                             | 2,955                    | 6.0                                            | 1,580                                    |
| 46.2                             | 3,355                    | 13.3                                           | 1,810                                    |
| 51.5                             | 3,650                    | 31.0                                           | 1,950                                    |
| 53                               | 3,738                    | 49.5                                           | 2,010                                    |
| 59                               | 3,800                    | 6.1 in. Hg                                     | 2,090                                    |
| 64.5                             | 4,200                    | 6.8                                            | 2,260                                    |
| 70.5                             | 4,550                    | 6.9                                            | 2,440                                    |

NOTE.—The above velocities are calculated from the formula

$$V = \frac{Q}{A}$$

when the normal area of oxygen passage 13 at burning end of nozzle is 0.074 sq. in. and with no regard to the acoustical velocity limitation which is about 982 for oxygen. Normal operating range during preheat period is 250 to 300 cubic feet/hour (about 135-161 feet/second through passage 13). Normal operating range during scarfing period is 2000 to 3000 cubic feet/hour (not to exceed 3500 cubic feet/hour), i. e., about 1080-1610 feet/second through passage 13.

In considering the novel process of thermochemically conditioning the surface of a hot ferrous metal body, according to the invention, it will be understood that the process comprises discharging acetylene from a series of outlets, in this case upper and lower slots 31, arranged in uniformly spaced relation to an edge of the body W and at the same time discharging streams of oxygen from orifices, in this case the oblong orifices 13, adjacent, i.e., between such acetylene outlets, to form a series of externally mixed oxy-acetylene flames. Such flames are applied against the body W in spaced parallel relation to such edge only until the temperature of the metal along such edge is raised to the ignition point. The surface S and such orifices are then moved with respect to each other; in the illustrated example the body W is moved in the direction of its length and with respect to the stationary nozzles N, as indicated by the arrow in Fig. 2. The velocity of all of the oxygen streams is then increased to a predetermined value for thermochemical reaction with such heated metal, preferably without changing the quantity of acetylene discharged from the outlets, so that each acetylene stream still is provided with sufficient oxygen at the point of exit of the acetylene from the orifices to form an externally mixed oxy-acetylene flame F adjacent, in this case above and below, said oxygen stream to provide the preheat flames needed for maintaining such thermochemical reaction. The relative movement between such orifices and the surface is such that the oxygen streams 14 and oxy-acetylene flames F thermochemically remove a layer of metal from the surface S of the body W.

In desurfacing a cold steel body, the latter is backed into position so that the post-mixed flames produced by the gases discharged from the nozzles are applied directly against the edge of the body. In either case, since the post-mixed oxy-acetylene flames contain an excess of oxygen, the starting zone becomes clearly visible as the metal reaches the kindling temperature, more quickly than in the case of premixed starting flames. This not only enables the operator to start the desurfacing movement of the body exactly at the proper instant, but reduces the starting period compared to that of premixed flames.

Furthermore, increasing the pressure of the oxygen supplied to the nozzles at the instant the desurfacing movement of the body is started, so that such body starts moving at the same instant the desurfacing streams are applied, inhibits gouging of the work surface in the starting zone.

The desurfacing or cutting action of the post-mixed desurfacing flames is more efficient than that of premixed flames, both in starting and in carrying on the operation, because the inner or primary combustion zones of the post-mixed flames are quite long and are applied close to the surface of the body. Since the greatest heat of an oxy-acetylene flame is adjacent the surface of the primary combustion zone or inner cone, it can be readily appreciated that the work is more effectively heated according to the present invention with post-mixed flames than with premixed flames. Furthermore, the shape of the post-mixed flames is somewhat bushy and luminous during the starting period when the oxygen

and acetylene are delivered to the nozzles in substantially equal volumes. When the oxygen streams are increased to a desurfacing velocity, however, at the end of the starting preheat period, the post-mixed preheating flames change in shape, becoming more non-luminous and well defined. In order to make the equipment as simple as possible, the quantity of acetylene supplied to the nozzles remains unchanged during the desurfacing operation, but it will be understood that the quantity of acetylene supplied to the nozzles may be changed in some cases without departing from the invention, should such change become necessary or desirable.

A beneficial feature of the present invention is the avoidance of flashbacks. This reduces the cost of maintenance and repair to a considerable extent. The equipment necessary to carry out the present process is very simple and inexpensive compared to that necessary for producing premixed flames. The present process removes metal faster, and the number of pounds of metal removed per cubic foot of oxygen is increased, so that the present process is more efficient than any prior desurfacing process. Another feature of the present invention is high stability, i.e., freedom from loss of cut, in the desurfacing operation. Another advantage of the present invention is the improvement in over-all efficiency of the desurfacing operation compared to those of the prior art. The surface resulting from the operation is of high quality, in which the ridges are almost flat.

As used in the following claims, the term "acetylene" is intended to cover any suitable combustible gas but not a mixture of such gases with a combustion-supporting gas. Also, as used in the claims, the term "externally mixed" means mixed outside of the blowpipe nozzle; and "post-mixed" means mixed after leaving the blowpipe nozzle.

We claim:

1. Process of thermochemically scarfing a ferrous metal body which is at a hot-rolling temperature, which process comprises discharging a substantially flat stream of commercially pure oxygen at a calculated velocity of 1000-1610 feet per second, simultaneously feeding thinner substantially flat upper and lower streams of commercially pure acetylene at acute angles directly into said stream of oxygen at a calculated velocity of about 240-267 feet per second, igniting the resulting mixtures of oxygen and acetylene, thereby producing a substantially flat stream of scarfing oxygen which is sandwiched between adjoining stable longitudinally extended upper and lower substantially flat post-mixed oxy-acetylene scarfing preheating flames having primary combustion zones which are about 1 and  $\frac{1}{4}$  inches long, applying the primary combustion zones of such flames and the scarfing oxygen stream at an acute angle directly against the surface of said body, and moving said body along a longitudinal path in a direction opposed to the flow of such stream, so that the body is thermochemically scarfed by such oxygen stream while the reaction is supported by said flames which also screen the scarfing zone from the atmosphere.

2. Process of thermochemically scarfing a ferrous metal body which is at a hot-rolling temperature, which process comprises discharging a substantially flat stream of commercially pure oxygen at a calculated velocity of about 135-161 feet per second, feeding thinner substantially flat upper and lower streams of commercially pure acetylene at acute angles into said stream of oxygen at a calculated velocity of 240-267 feet per second, igniting the resulting substantially flat stream of mixed oxygen and acetylene, thereby producing outside of the nozzle a relatively long oxidizing post-mixed substantially flat starting preheating flame having a primary combustion zone extending about 1 and  $\frac{1}{4}$  inches from said nozzle, applying the primary combustion zone of such preheating flame directly against the surface of said body with the transverse axis of the flame parallel and the longitudinal axis of the flame at an acute angle to such surface, holding said body substantially stationary until the hot ferrous metal is further

heated by such flame sufficiently to be ignited by the excess oxygen of such flame, and thereupon simultaneously starting to advance said body along a path parallel to the surface of the body, and increasing the flow of oxygen to increase the velocity of the discharged oxygen stream to a calculated velocity of about 1000-1610 feet per second while maintaining the flow of acetylene at a calculated velocity of about 240-267 feet per second, thereby producing a scarfing stream of oxygen which is substantially flat and is sandwiched between adjoining stable extended upper and lower post-mixed oxy-acetylene scarfing preheating flames which have hard primary combustion zones which are in direct contact with the surface of the body, and thermochemically scarfing the ferrous metal body therewith by movement of the body along such path.

3. Process of scarfing a hot ferrous metal body, as defined by claim 2, in which a plurality of such streams are similarly operated in side-by-side relation so that the preheating flames and streams of scarfing oxygen merge laterally to preheat and scarf a relatively wide area of the body in a single pass.

JAMES H. BUCKNAM.  
IVAN P. THOMPSON.

#### REFERENCES CITED

30 The following references are of record in the file of this patent:

#### UNITED STATES PATENTS

| Number       | Name     | Date           |
|--------------|----------|----------------|
| 35 703,940   | Menne    | July 1, 1902   |
| 968,350      | Harrison | Aug. 23, 1910  |
| 1,311,815    | Harris   | July 29, 1919  |
| 1,519,582    | Harris   | Dec. 16, 1924  |
| 1,957,351    | Oldham   | May 1, 1934    |
| 40 2,210,402 | Gaines   | Aug. 6, 1940   |
| 2,215,577    | Bucknam  | Sept. 24, 1940 |
| 2,267,405    | Jones    | Dec. 13, 1941  |
| 2,290,295    | Scheller | July 21, 1942  |

#### FOREIGN PATENTS

| Number  | Country       | Date          |
|---------|---------------|---------------|
| 11,380  | Great Britain | July 22, 1915 |
| of 1914 |               |               |
| 617,256 | France        | Nov. 19, 1926 |
| 817,708 | France        | May 31, 1937  |